

Oct. 27, 1953

N. W. F. PHILLIPS ET AL

2,657,118

METHOD OF PURIFYING CARBONACEOUS MATERIAL

Filed Sept. 21, 1950



Norman W. F. Phillips  
Ethan Hollingshead  
James S. Mutchmor  
INVENTOR.

BY Robert S. Dunham

ATTORNEY

## UNITED STATES PATENT OFFICE

2,657,118

## METHOD OF PURIFYING CARBONACEOUS MATERIAL

Norman W. F. Phillips, Ethan A. Hollingshead, and James S. Mutchmor, Arvida, Quebec, Canada, assignors to Aluminum Laboratories Limited, Montreal, Quebec, Canada, a corporation of the Dominion of Canada

Application September 21, 1950, Serial No. 185,947

14 Claims. (Cl. 23—209.9)

1

This invention relates to the purification of coke and coal, viz., carbonaceous material of coal origin, and is particularly directed to the manufacture, from such material, of a purified carbon having a greatly reduced content of so-called ash, i. e. inorganic impurities of which important examples are iron and silicon. In a more specific sense, the invention is directed to the treatment of coke or anthracite coal for conversion into a carbon product having such purity and other characteristics as to be suitable for making carbon electrodes which can be used in electrolytic procedures of the molten electrolyte type.

For example, in the manufacture of aluminum by electrolytic reduction of alumina in a suitable fused bath, the necessary carbon electrodes have usually been manufactured from so-called petroleum coke, of relatively high purity. In order to obtain metallic aluminum having a very low content, if any, of elements such as iron, silicon, titanium and the like (e. g. aluminum with at most a few tenths of a percent total impurity), it is essential that the electrodes be relatively free of such elements; that is to say, the electrodes are continuously consumed in the operation and any impurities of this character pass into the bath and thence go to contaminate the deposited aluminum. Although petroleum coke may sometimes be unavailable or unavoidably costly, ordinary coke, anthracite coal and the like have not heretofore been economical substitutes for carbon electrode manufacture, because of their high content of impurities of the character stated. It may be noted, in passing, that references herein to "coke" mean ordinary coke derived from coal (usually bituminous coal) unless otherwise specifically designated.

Accordingly, chief objects of the invention are to afford improved procedure for purifying materials of this class (coke and coal), notably procedure which is of a simple, efficient and economical character and which yields a greatly purified carbon product, especially one that is suitable for making electrodes of the sort mentioned above. A specific object of the invention is to afford new, improved and more effective methods of purifying such material, particularly coke, by chlorination.

To these and other ends, it has now been discovered that a fully sufficient and indeed relatively complete separation of the impurities from coke or like material may be achieved by treating it with chlorine gas at the critically elevated temperature of about 1400° C. or higher, for a reasonable period of time. By such treatment

5 the total ash content of coke can be reduced from a value of 10% or more to 2% or less, the most difficultly separable contaminants, such as iron and silicon being removed to the point where only a minor fraction of a percent of each remains (all such percentages being given by weight, herein). The process is advantageously carried out by flowing chlorine gas through the coke or coal while heating the latter to keep it in the stated, extremely high temperature range. Good results can be obtained in even a very few hours, and in all cases within a period that permits economical and efficient operation. According to present understanding, the chlorine reacts with materials such as iron oxide, silica and titanium oxide to yield volatile chlorides of the metals. The chlorides are in fact formed or immediately released in a volatilized or gaseous state and are swept out of the treatment zone in the current of gas flow. The following equations 10 are understood to represent the type of reaction which thus occurs between the contaminating metal compounds and chlorine in the presence of carbon, all of the reaction products being established and separated in the gaseous state:



30 While treatment of coke with chlorine at moderately high temperatures, e. g. up to 1100° C. or so, has been heretofore proposed with the view of purifying the material by reactions of this sort, experience has indicated that such treatments are ineffective to produce a satisfactorily pure carbon, and specifically are incapable of yielding a reduction of silica content suitable for highly pure electrode carbon or of yielding such reduction in any reasonably rapid and efficient manner. It has neither been apparent nor recognized, however, that operation at substantially greater temperatures would afford significant improvement in such results or would aid them in any workable manner or within an economically feasible time of treatment. Indeed there seemed no practical way of obtaining a suitably pure carbon from coke by the previously suggested chlorination methods (even up to 1000°–1200° C.) except perhaps by subjecting the coke, after such treatment, to the action of hydrofluoric acid. For instance, by applying gaseous hydrogen fluoride at a suitably high temperature, much of the silicon content can be converted to a volatile fluoride, but such operation is costly, and very inconvenient because of the corrosive or reactive 35 nature of hydrofluoric acid. With the process of

## 3

the present discovery, there is ordinarily no need for a supplemental fluoride treatment; on the contrary, an unusually complete separation of silicon, as well as improved purification with respect to other mineral impurities (e. g. iron, titanium and the like), can be achieved by a single, economical operation.

In carrying out the method in a manner that now seems most practical, the coke, in a suitably granular state, is charged into a furnace having appropriate means for heating the charge and for the continuous traversal of gas. Chlorine gas is continuously introduced, say at the bottom of the furnace, and the spent gas containing the reaction products is continuously withdrawn at the top, so that a constant flow of chlorine permeates the coke which is kept at the selected high temperature in the reaction zone. One effective expedient is to heat the charge electrically by its own resistance, e. g. by passing a current through the body of coke between electrodes which project into it. The temperature of at least the main body or major part of the coke in the reaction zone is kept at 1400° C. or more, the hottest parts of the charge probably reaching 1600° to 1700° C. or so. Present evidence does not indicate that there is any specific upper limit to the temperature, beyond such as may be imposed by economy and convenience. Under conditions appropriate to commercial operation and with cokes of average character, amply satisfactory results have been obtained where the temperature is in the range stated; at an extremely high heat (say, if the bulk of the charge is heated to above 1600° C.), energy requirements and adverse effects on the furnace structure are apt to be objectionable.

While considerable conversion of metallic impurities to volatile chlorides can be achieved by treatments not greatly exceeding one hour, a chlorination period of several hours is ordinarily desirable, to decrease the silica and other contamination of the coke to usefully low values. In the case of large quantities of coke, the treatment at 1400° to 1500° C. should preferably have a duration of the order of 6 to 10 hours; for instance, with large furnaces operated on a semi-continuous basis, the total passage time for any specific quantity of coke through the pre-heating, reaction and discharge zones may be as much as 12 hours or more, yet without detriment to the efficiency of the operation. It will be understood that such a furnace is advantageously arranged to permit some pre-heating of the coke by conduction and by the effluent gas, before it reaches the region of direct heating. As explained, chlorine gas flows continuously into the furnace, very preferably in a direction countercurrent to the travel of coke although concurrent operation can be employed in some cases.

Upon completion of the desired period of treatment with a given batch or portion of coke, it may be discharged from the furnace and appropriately cooled or quenched to prevent its burning and to permit its being handled in conventional conveying equipment. For example, dry cooling, as by combustion or other inert gases (if available) can be employed, or more conveniently in most cases, a quenching operation can be performed with a water spray and preferably in such fashion that the product is not left in a wet condition. While there is usually some chlorine in the product, such contamination is significantly less in the present process than has been found in prior chlorination treatment at temperatures

## 4

of 1000° to 1100° C. This difference in chlorine contamination has been particularly noted in the case of anthracite coal; while treatment of such material at 1000° C. leaves a relatively considerable chlorine content, treatment in accordance with the present invention leaves only a much smaller amount of chlorine in the coal.

In any case, it has been found that if the chlorine content of the coke or coal is too high, it may be simply and effectively reduced by treatment with hydrogen. For instance by treating the chlorinated coke or anthracite in a furnace at 1400° C. with a moderate flow of hydrogen gas for one to three hours, chlorine concentrations of 0.8 to 1.1% in such products have been lowered to 0.3 to 0.5%.

By way of illustration of the results of the present process and also to show its advantage in comparison with chlorination treatment effected at a lower temperature, the following are representative examples of many tests which were conducted with various kinds of coke and anthracite coal. The reaction vessels were vertically disposed, porcelain tubes surrounded by electrical resistance furnaces to heat the contained charge, i. e. granular coke or anthracite which was supported on a perforated graphite plate in the lower end of the tube. A metered stream of chlorine was introduced at the bottom of each tube, while the volatile chlorides and carbon monoxide were withdrawn from top. In the case of such treatments of two cokes of ordinary but separate commercial origin (respectively designated as A and B, and each derived from bituminous coal) and like treatment of samples of a Welsh anthracite coal, the following table shows the pertinent impurity concentrations (total ash, and iron, silicon and titanium separately) of the untreated material and of materials treated in tests at the several temperatures respectively and for the times of treatment stated. Each operation at a specified temperature represented the separate treatment of a fresh 200 gram sample of material. In each case, the coke or anthracite had a particle size such that the grains would pass a screen with a 0.3 inch opening and remain on a screen with a 0.15 inch opening, and the chlorine was supplied at the rate of one liter per minute throughout the time specified.

## 50 Chlorination of coke and anthracite batches

|                            | Per-cent Ash | Per-cent Fe | Per-cent Si | Per-cent Ti | Per-cent Cl |
|----------------------------|--------------|-------------|-------------|-------------|-------------|
| Untreated coke A           | 11.7         | 0.73        | 2.13        | 0.08        |             |
| After 3 hr. at 1200° C.    | 3.9          | 0.54        | 0.69        | 0.05        |             |
| After 3 hr. at 1400° C.    | 2.1          | 0.30        | 0.19        | 0.05        |             |
| Untreated coke B           | 13.0         | 0.87        | 3.02        | 0.10        |             |
| After 3 hr. at 1200° C.    | 6.3          | 0.38        | 1.50        | 0.06        |             |
| After 3 hr. at 1400° C.    | 1.4          | 0.26        | 0.22        | 0.05        |             |
| Untreated Welsh anthracite | 2.4          | 0.24        | 0.46        | 0.01        | 0.01        |
| After 12 hr. at 1000° C.   | 1.0          | 0.05        | 0.16        | 0.01        | 5.5         |
| After 12 hr. at 1200° C.   | 1.2          | 0.05        | 0.26        | 0.02        | 2.8         |
| After 12 hr. at 1400° C.   | 0.7          | 0.05        | 0.04        | 0.01        | 1.9         |

The last operation in each set of the above, i. e. at 1400° C., represented the process of the present invention, which in the case of the cokes afforded a great improvement over lower temperature treatment, in reducing the silicon contamination, as well as in providing a product of very low total ash content and appropriately low concentration of iron and titanium. Likewise, in the case of anthracite coal, a very marked reduction in silicon content was obtained, it being also noted that the chlorine content remaining after treatment by the pres-

ent process was much less than after the operations at 1000° or 1200° C. It should be remarked that this specific type of anthracite had an unusually low total ash content, and that the advantages of the invention are even more fully realized, for treatment of coal, in the case of Pennsylvania or other anthracite having a relatively high ash, including correspondingly high content of the various impurities specifically noted above.

The accompanying drawing is a diagrammatic view of a furnace employed in carrying out the process, shown in central, vertical section, the drawing also serving to illustrate the process itself. While other types of furnace may be used, the arrangement shown has been found very effective. Essentially, the apparatus comprises a vertical shaft furnace housed in a gas-tight steel shell 10 and lined with refractory material 12, preferably dense, high quality fire-clay or like refractory (in brick, tile or other form), usually or preponderantly having a composition of aluminum silicate or silicates. Portions of coke or anthracite to be treated are added at the top 13 and portions of purified coke product are withdrawn from the bottom 14, from time to time, so that the cylindrical furnace chamber 15 is always substantially filled with coke 17, intermittently moving downward. Chlorine gas is introduced continuously through a lower inlet 18 and spent gases removed from an upper outlet 19. Although other heating means can be used, the coke charge is preferably heated by internal means, and very advantageously by the resistance heating effect of electric current traveling through the charge, as between one or more upper carbon electrodes 20 and one or more lower carbon electrodes 21, the illustrated furnace having three such electrodes (of which two are shown) at each locality, all extending well into the furnace. Thus the electric current or currents are conducted through the coke, along paths essentially parallel to the furnace wall 12 and to the directions of countercurrent travel of the coke and chlorine gas, the great preponderance of the current and hence of the heating effect being disposed inwardly of the furnace wall.

As another example of the invention, coke was treated in a vertical shaft furnace of the character shown and having an internal diameter of 4.5 feet, lined with refractory material and provided with carbon electrodes 20, 21 arranged for passage of current through the coke charge in a vertical direction, e. g. over a distance of the order of 20 feet. The coke was in the form of large grains, having rather uniformly a size of about  $\frac{3}{8}$  inch diameter. With the heated zone capacity of the furnace being about 6 tons, and with chlorine passed through the heated charge at rates varied from about 100 to about 300 pounds per hour, purified coke was produced at the rate of 250 to 500 pounds or more per hour. Quantities of raw coke were added at the top of the furnace and quantities of purified product withdrawn from the bottom at regular intervals, the production rate of suitably pure carbon being found to vary roughly with the rate of chlorine supply, within the ranges mentioned. The average analysis of the supplied coke indicated a total ash content of 10%, specific impurity concentrations (measured in each case as the designated element) being 0.8% iron, 2.2% silicon and 0.2% titanium. Approximately 50 tons of suitably purified carbon product, made

in a number of runs as just described, contained on the average and with reasonable uniformity: 1.2% total ash; 0.10% iron, 0.10% silicon and 0.03% titanium.

While a longer actual treatment time for a given portion of coke was employed in some of these runs and may sometimes be more economical in continuous production, it was found that a contact time of 8 to 12 hours at the specified temperature and with chlorine flow preferably at the higher end of the range last above mentioned, will usually assure production of a purified carbon having well under 0.2% iron, well under 0.2% silicon and less than 0.05% titanium. It will now be appreciated that the conditions of operation in any given case should and easily can be selected to suit the specific circumstances, including the average analysis of the coke used and the specific purity desired in the product. The process can be successfully run so that there is little or no free chlorine in the effluent gas; economical results of this type were obtained in the several furnace operations described herein, at least 50% of the supplied chlorine being consumed in actual reaction with various components or constituents of the ash content of the coke. Some of the chlorine is unavoidably lost in attack on the refractory lining of the furnace (which must be re-surfaced or renewed from time to time) and a small proportion may be retained in the coke, as explained above, but the operation has proved amply efficient in yielding a pure, electrode-type carbon at reasonable cost.

In a modified furnace of the same upright shaft type and electrical heating arrangement (illustrated in the drawing), but having a thicker lining of refractory brick and thus an internal diameter of 3 feet, like results were obtained. This furnace had a total holding capacity of 4.7 tons of coke, including 2.8 tons in the heated zone. The raw coke had an ash content of about 9%, including about 0.6% Fe, 2.0% Si and 0.08% Ti. With the temperature of the charge at 1400° C. (and higher at the center) and with chlorine supplied at 94 lbs. per hour, which equalled 0.36 lb. of chlorine per pound of product, a production rate of over 3 tons per day (of 24 hours) was achieved. The ash content of the product was about 2%, including 0.09% iron, 0.15% silicon, and 0.04% titanium. At a slightly lower production rate and with a little less chlorine a purified coke was obtained having only 0.66% total ash, 0.05% Fe, 0.07 Si and 0.04% Ti.

When anthracite coal is treated in a furnace which is to be heated by passage of electric current through the charge, it is usually desirable to perform first at least a partial calcination, e. g. by pre-heating the coal with the exhaust gases and by conduction in an upper part of the furnace, in order to reduce the resistance of the coal to a value permitting sufficient flow of current. In a continuous operation on anthracite, it will be understood that the furnace can be filled at the outset with coke or with anthracite which has been suitably calcined; thereafter, subsequently introduced quantities of the coal are sufficiently pretreated in the upper part of the furnace before descending to the principal reaction zone.

In the examples of furnace operations, the temperature was maintained at 1400° C. or higher throughout nearly all of the charge between the electrodes, i. e. except for a small part at lower temperature immediately adjacent the refractory wall. No very critical regulation was employed

or found necessary. As stated above, it was apparent that the temperature in the center or hottest part of the charge was considerably higher, probably reaching 1600° C. or more. It was found desirable, to avoid hydrolysis of volatile chlorides with moisture in the coke entering the top of the furnace, that the coke have a moisture content of not more than about 0.5%, such condition being achieved by preliminary drying if necessary. Direct condensation of chlorides in the entering coke was satisfactorily avoided by adding small amounts of coke frequently rather than larger quantities less often, and by keeping the charge level at not more than a certain distance (compatible with heat economy) above the uppermost current-supplying electrodes, e. g. 8 feet in the larger of the above furnaces and 3 feet in the smaller. In these ways, deposition of finely divided solids in the interstices of freshly charged coke was avoided; while such material would presumably be eliminated in the high temperature zone, it sometimes tended to impede proper downward flow or charging of the coke, or to have a clogging effect against a desirably high rate of gas passage. When necessary, preliminary cleaning or like treatments of a conventional sort may be performed on the coke or on the coal from which it is made, such as tabling operations or other physical beneficiation, to separate particles or pieces of foreign matter prior to the present process.

A particularly important feature or attribute of the process, especially when carried out in a furnace for example of the type shown, is that the carbonaceous charge exhibits a surprisingly high temperature gradient in regions close to and adjoining the inside furnace wall. Thus it was discovered that in the present procedure, notably when performed with internal heating of a coke charge, the temperature gradient next to the fire-clay brick wall (i. e. the inner surface of the wall 12 in the drawing) is about 200° C. per inch, a condition that was unexpected in view of the relatively high thermal conductivity of coke. Indeed, evidence indicates that where the average temperature of the charge is 1400° C. or more and the temperature at the center may be as high as about 1600° C., the temperature begins to fall off rapidly (when considered radially outward from the center of the furnace toward the wall) at say, several inches from the wall, and reaches the stated, very high gradient at the outermost localities of the charge body. A notable advantage of this condition is that the deterioration of the furnace, especially by chemical attack, is greatly reduced; that is to say, at temperatures well below 1400° C. and especially at about 1200° C. (or less), the rate of attack of furnace gas (i. e. chlorine) on the refractory material is much less than at 1400° and higher.

Thus the process may be effectively performed (in a zone advantageously lined with refractory) with essentially all of the charge at the desired, high temperatures and yet with an economically low rate of attack or disintegration of the furnace lining, i. e. very considerably lower than if such refractory material (aluminum silicates) or the like were subjected to temperatures in the range of 1400° to 1600° or so. At the same time, the small portion or layer of coke that adjoins the wall tends to travel downward more slowly than the main body of the charge, and thus even this layer somewhat tends to be compensated, by a longer time of treatment, for the slower purification there occurring. The advantageous and

unusually high temperature gradient at the periphery of the charge does not seem to depend significantly on the chemical composition of lining, except that it has been fully realized in furnaces having a lining of conventional dense refractory, and may be less where a large amount of porous or other highly insulating material is used and provides for a large temperature drop, between the reaction chamber and the outer steel shell. As indicated above, the peripheral gradient in the coke or anthracite is enhanced, or very significantly effectuated by procedure involving internal heating of the charge, especially by the passage of electric current in the manner described above in reference to the drawing. Thus the supplied current is easily controlled to heat the major part of the coke charge to the desired temperature of 1400° C. or so, i. e. so that the average temperature of the charge is at such temperature or higher, yet with insufficient heating effect (due to the stated gradient) to heat the refractory lining above about 1200° C.

It will now be seen that the described procedures of the invention afford economical and efficient operations for the purification of coal-type material to obtain a carbon product suitable for various uses, especially for the manufacture of carbon electrodes. The method is peculiarly effective in the case of coke and anthracite coal. In fact it is usefully capable of removing inorganic ash material (e. g. iron, silicon or the like) from bituminous coal, but the properties of this material when heated ordinarily render its treatment difficult and uneconomical. Therefore while some bituminous coals, especially types having characteristics somewhat approaching those of anthracite, might be successfully treated, bituminous coal is not in general now considered a preferred raw material for the process described herein.

It is to be understood that the invention is not limited to the specific procedures hereinabove described but may be carried out in other ways without departure from its spirit.

We claim:

1. A method of purifying carbonaceous material of coal origin which contains inorganic contaminating material, comprising treating the carbonaceous material with chlorine at a temperature of at least about 1400° C. to convert inorganic contaminating material to volatilized form, and separating the volatilized material from the carbonaceous material.

2. A method of purifying silicon-containing carbonaceous material of coal origin, comprising treating the material with chlorine at a temperature of at least about 1400° C. to convert silicon contained in said material to volatilized, compound form, and separating the volatilized silicon compound from the material.

3. A method of purifying material of the class consisting of coke and anthracite coal, said material containing inorganic impurities including at least 0.4% silicon, comprising treating the material with chlorine at a temperature of at least about 1400° C., to reduce the silicon content of the material to less than 0.2% by converting impurities in the material, including silicon, to volatilized form, and separating the volatilized impurities from the material.

4. A method of purifying material of the class consisting of coke and anthracite coal to reduce the content of iron and silicon in said material, comprising treating the material with chlorine at a temperature of at least about 1400° C. for at least three hours, to convert impurities in the

material, including iron and silicon, to volatilized form, and separating the volatilized impurities from the material.

5. A method of purifying coke containing impurities constituting an ash content of more than 5%, comprising treating the coke by passing chlorine gas through it while maintaining the coke at a temperature of at least about 1400° C., to reduce the ash content to not more than about 2% by converting impurities in the coke to volatilized form, said volatilized impurities being carried away from the coke with the passing gas.

6. A method of purifying coke which contains impurities including more than 0.5% iron and more than 1% silicon, comprising continuously passing chlorine gas through a body of the coke having a moisture content of not more than 0.5% while maintaining the coke at a temperature of at least about 1400° C., to reduce the iron and silicon content to not more than about 0.2% each by converting impurities in the coke, including iron and silicon, into volatilized form, said volatilized impurities being carried away from the coke with the passing gas.

7. A method of purifying inorganic impurity-containing carbonaceous material of coal origin, comprising treating the material with chlorine at a temperature of at least about 1400° C. for at least about six hours, to convert inorganic impurities in the material into volatilized form, and separating the volatilized impurities from the material.

8. A method of purifying coke which contains impurities including iron and silicon, comprising treating the coke with chlorine at a temperature of at least about 1400° C. for at least eight hours, to convert impurities in the material, including iron and silicon, into volatilized form, separating the volatilized impurities from the coke and recovering the purified coke.

9. A method of treating carbonaceous material of coal origin to purify it, comprising passing chlorine gas through a body of said material which is laterally confined at a boundary that extends around the body, and heating a major part of the body to at least about 1400° C. during said passage of chlorine, while maintaining a temperature gradient in the outermost portion of the material adjacent said boundary, and thereby keeping the temperature of the material at said boundary at a value substantially below 1400° C.

10. A method of treating coke to purify it, comprising passing coke in divided form downward through a vertically elongated reaction zone peripherally lined with dense refractory material, while passing chlorine gas upward through said zone, and heating the coke so that a major part of the coke is heated to a temperature of at least about 1400° C. during said passage of chlorine, while maintaining a sharp temperature gradient in the coke near the periphery of the zone, decreasing toward said periphery, and thereby preventing the temperature of the coke at said periphery from rising above about 1200° C.

11. A method of treating coke to purify it, comprising passing chlorine gas through a body of coke in permeable form, while confining the body of coke within a surrounding surface and while heating the body of coke by releasing heat internally thereof at localities which are at least nearly all spaced internally of the body from said surface, said heat being sufficient to heat a

major part of said body to at least about 1400° C., while maintaining a temperature gradient in the portion of the coke immediately adjacent said surface, so as to prevent the temperature of said surface from rising higher than about 1200° C.

12. A method of treating carbonaceous material of coal origin to purify it, comprising passing said material in divided form through an elongated reaction zone peripherally lined with dense refractory material, while passing chlorine gas through said zone, and while passing electric current through the material in said zone between terminal regions spaced lengthwise of the zone and lying principally in the path of the material, so that a major part of the material is heated to a temperature of at least about 1400° C., a temperature gradient decreasing toward the periphery of the zone being maintained in the material near said periphery, and the aforesaid heating of the material by the current being effected so that by said gradient the temperature of the material at said periphery is kept substantially below 1400° C.

13. A method of treating coke to purify it, comprising passing successive quantities of coke in divided form downward through a vertically elongated reaction zone wherein the coke is laterally confined at a predetermined boundary, while passing chlorine gas upward through said zone, and while heating a major part of the coke in said zone to at least about 1400° C. by passing electric current through the coke, at least nearly all of said current being passed along paths distributed in a region of the zone spaced centrally inward of said boundary, a temperature gradient decreasing toward said boundary being maintained in the coke near said boundary, and the heating of the coke by the current as aforesaid being controlled to prevent the temperature of the coke at said boundary from rising above about 1200° C.

14. A method of treating coke to purify it, comprising passing chlorine gas through a body of coke which is laterally confined at a boundary that extends around the body and lengthwise thereof in a predetermined direction, said coke being in divided form, and heating a major part of the body to at least about 1400° C. during said passage of chlorine, by passing electric current through said coke, at least nearly all of said current being passed along paths distributed in a region of the body spaced centrally inward of said boundary, a temperature gradient decreasing toward said boundary being maintained in the coke near said boundary, and the heating of the coke by the current as aforesaid being controlled to prevent the temperature of the coke at said boundary from rising above about 1200° C.

NORMAN W. F. PHILLIPS.

ETHAN A. HOLLINGSHEAD.

JAMES S. MUNCHIMOR.

References Cited in the file of this patent

UNITED STATES PATENTS

| Number    | Name                    | Date          |
|-----------|-------------------------|---------------|
| 1,071,442 | Lee _____               | Aug. 26, 1913 |
| 1,271,713 | Hutchins _____          | July 9, 1918  |
| 1,277,707 | Dyrssen _____           | Sept. 3, 1918 |
| 1,303,362 | Mott _____              | May 13, 1919  |
| 1,671,673 | Doerscheek et al. _____ | May 29, 1928  |
| 2,260,746 | Hanawalt et al. _____   | Oct. 28, 1941 |
| 2,315,346 | Mitchell _____          | Mar. 30, 1943 |